

# UNITED STATES PATENT OFFICE.

CHARLES MORRIS JOHNSON, OF AVALON, PENNSYLVANIA.

## ALLOY STEEL.

1,420,708.

Specification of Letters Patent. Patented June 27, 1922.

No Drawing.

Application filed March 28, 1921. Serial No. 456,191.

To all whom it may concern:

Be it known that I, CHARLES MORRIS JOHNSON, residing at Avalon, in the county of Allegheny and State of Pennsylvania, a citizen of the United States, have invented or discovered certain new and useful Improvements in Alloy Steel, of which improvements the following is a specification.

In a prior application filed by me on August 9th, 1920, Serial No. 401,656, I described a new alloy steel containing chromium, nickel and silicon, which I had found to be strongly resistant to high heat, to acids, and to rust, while at the same time being non-magnetic. Stated generally, the said steel contained from about ten per cent to about twenty per cent of chromium, from about nine per cent to about twenty-five per cent of nickel, and from about one per cent to about ten per cent of silicon, but it was considered preferably that the chromium and the nickel should be contained in the steel in fairly equal proportions. Such steel, as is stated in the said application, was very tough, and was consequently somewhat difficult to machine.

In making further investigations with a view to enlarging the field of usefulness of the steel of my aforesaid application, I have discovered that a steel of this type can be rendered easily machinable by changing the relative proportions of the chromium and nickel contents, that is to say by using nickel in amount substantially double the amount of chromium; or even greatly in excess of double,—in some cases, where hardness is of minor importance, the content of nickel may be even six times the chromium content,—the silicon content being in general subject to the same variations as in the steel of my said prior application. This change in the relative proportions of the chromium and nickel results in a lowering of the chromium limit and an increasing of the nickel limit, as compared with said prior steel. Thus in this case the chromium in the steel may range from about six per cent to about eighteen per cent, and the nickel from about twelve per cent to about thirty-six per cent, while the silicon content may be from about one per cent to about ten per cent as before. In any case the iron should be kept at a

minimum of fifty per cent of the product, in order to insure tensile strength, and to obtain a steel which can be forged, rolled and drawn, as may be required. As before, the carbon will ordinarily be less than one per cent, and in most cases less than one-half of one per cent.

Within the above limits I have produced steel containing chromium from ten per cent to fifteen per cent, nickel from thirty per cent to thirty-six per cent, silicon about four per cent, and carbon from .30 per cent to .50 per cent, which is easily machinable, while possessing to an extent sufficient for many purposes all of the resistant qualities of the steel of my said prior application. This steel, as well as that of my said prior application, is of high electrical resistance, and is therefore useful in varieties of electrical apparatus where that quality is desired.

It is a matter of common experience that nickel and cobalt have many like chemical properties, and that the metallurgical effects in alloy steels are generally alike, so I desire it to be understood that in the appended claims I intend to cover the use of cobalt as a substitute for nickel in whole or in part. The steel may of course contain the usual small quantities of manganese, etc., and other alloying elements may also be employed without departure from the invention.

I claim as my invention:

1. Steel containing from about six per cent to about eighteen per cent of chromium, from about twelve per cent to about thirty-six per cent of nickel, from about one per cent to about ten per cent of silicon, and at least fifty per cent of iron, the content of nickel being substantially double (or more) the content of chromium.

2. Steel containing from ten per cent to fifteen per cent of chromium, from thirty per cent to thirty-six per cent of nickel, from one per cent to five per cent of silicon, and not less than fifty per cent of iron.

In testimony whereof I have hereunto set my hand.

CHARLES MORRIS JOHNSON.

Witnesses:

MARSHALL A. CHRISTY,  
FRANCIS J. TOMASSON.